

# United States Patent [19]

Boyars et al.

[11] 3,775,199

[45] Nov. 27, 1973

[54] NITROGEN GENERATOR

[75] Inventors: Carl Boyars; Carl T. Zovko, both of Silver Spring, Md.

[73] Assignee: The United States of America, as represented by the Secretary of the Navy, Washington, D.C.

[22] Filed: Oct. 13, 1972

[21] Appl. No.: 297,513

[52] U.S. Cl. .... 149/35, 149/74

[51] Int. Cl. .... C06c 1/02

[58] Field of Search .... 149/35, 74; 252/5, 252/7

[56] References Cited

UNITED STATES PATENTS

2,981,616 4/1961 Boyer..... 149/35

Primary Examiner—Stephen J. Lechert, Jr.

Attorney—R. S. Sciascia et al.

[57] ABSTRACT

A material for generating hot nitrogen gas comprising sodium azide and sulfur in the presence of a conventional solid propellant ignitor.

14 Claims, No Drawings

## NITROGEN GENERATOR

## BACKGROUND OF THE INVENTION

This invention generally relates to a gas generator and more particularly to a solid propellant nitrogen gas generator.

Currently nitrogen gas generators find use in the fields of electric power, mechanical work, pressurization of liquid propellants and as a fuel source for gas dynamic lasers. Gas dynamic lasers utilizing gas compositions which are mainly  $N_2$ , have been operated by arc heating of the gas, which had been stored as a gas under pressure or as a cryogenic liquid or else by the combustion of pre-heated CO with  $O_2$ , with subsequent addition of  $N_2$  from the same sources. However, any system of furnishing the gas composition which depends on pressurized or cryogenic  $N_2$  is undesirably bulky and inconvenient.

Some nitrogen gas generators are based on the reaction of  $NaN_3$  with  $F_2$ ,  $ClF_3$ ,  $N_2O_4$  or other similar materials to produce  $N_2$  but use of these toxic, corrosive gases and liquids have proven to be unacceptably hazardous to personnel.

Thus research has been conducted in an attempt to find a relatively safe method of producing nitrogen which does not require the use of bulky, inconvenient equipment.

## SUMMARY OF THE INVENTION

Accordingly one object of this invention is to provide a new composition for generating nitrogen.

Another object of this invention is to provide a composition for generating nitrogen which is not bulky, and inconvenient to use.

A still further object of this invention is to provide a composition for generating nitrogen which does not use toxic or corrosive materials which are hazardous to personnel.

Yet another object of this invention is to provide a composition for generating pure nitrogen which can be used in gas dynamic lasers.

A still further object of this invention is to provide nitrogen which can be used in the fields of electrical power, mechanical work and pressurization of liquid propellants.

These and other objects of this invention are accomplished by providing a solid composition comprising sodium azide or an azide of similar sensitivity, and sulfur which are in the presence of a conventional solid propellant initiator.

## DESCRIPTION OF THE PREFERRED EMBODIMENT

The present invention comprises a solid composition which is capable of producing hot nitrogen gas. This composition comprises (1) sodium azide or an azide of similar sensitivity and (2) sulfur which are in the presence of any of the conventional solid propellant initiators. If it is desired to have  $CO_2$  present together with the nitrogen gas, as is the case when  $N_2$  is used in gas dynamic lasers wherein it is desirable for the gas being generated to comprise about 80-90 percent  $N_2$ , 10-15 percent  $CO_2$ , and 1-2 percent water, the  $CO_2$  may be added after  $N_2$  generation or it may be supplied by adding a carbonate or other fuel oxidizer combinations such as carbon and sodium nitrate to the solid propellant.

Since the azide and sulfur are not hypergolic it is necessary to have an initiator or ignitor present in the combustion chamber in order to start the reaction. The reaction is started by burning or otherwise igniting a small conventional solid propellant ignitor. Once the reaction has started the ignitor is no longer necessary. Once started the stoichiometric reaction between sodium azide and sulfur is



In situations where it is desirable to have as few products in addition to  $N_2$  present in the gas, it is preferred to have about stoichiometric amounts of the azide and sulfur present. However for most uses, it is only necessary to have some quantity of the fuel and oxidizer present. In practice where low combustion temperatures are desirable to minimize impurities in the gas, it is preferable to have the sulfur constituent present in an amount less than stoichiometric, even as low as 20 percent of the stoichiometric quantity, and preferably as low as about 75 percent of the stoichiometric quantity. As will be recognized by those skilled in the art, it is also desirable to have the azide constituent present in an amount no less than 20 percent of the stoichiometric quantity and preferably as about 75 percent of the stoichiometric quantity.

As can be seen from the above equation, the chemical reaction that produces  $N_2$  also produces other products. For some uses, such as gas dynamic laser, these impurities should be removed before the gas enters the laser, because impurities of this type can plug the nozzle, absorb or scatter light or coat the optical components. The solid and/or liquid impurities can be removed by any of the conventional techniques such as, for example, by passing the gas through a series of baffles while the gas is still at high pressure and low velocity. The entrained particles will not follow the same path as the gas stream and they will impinge on the walls and be trapped.

It should be noted that other azides beside sodium azide may be used in the compositions of this invention provided that the azide has a similar sensitivity to sodium azide. A specific azide which may be used is lithium azide.

The conventional solid propellant ignitor which is used to initiate reaction need only be present in extremely small quantities because once the reaction is started it no longer requires the presence of the ignitor. Any of the well known solid propellant ignitors can be used. Some examples of these ignitors are black powder, pyrotechnics, metal oxidant mixtures, such as boron/ $KNO_3$ , aluminum/potassium perchlorate, thermites, etc. The exact nature of the ignitor is immaterial since its only function is to start the reaction. Thus the ignitor is a separate device which contains any of the art recognized solid propellant initiators and which is either contained in or vented into the combustion chamber.

The general nature of the invention having been set forth, the following example is presented as a specific illustration thereof. It will be understood that the invention is not limited to this example but is susceptible to various modifications that will be recognized by one of ordinary skill in the art.

## EXAMPLE

A 20 gram pellet of 80 percent by weight  $NaN_3$  and

20 percent by weight S was prepared. About 2 grams of the standard solid rocket propellant initiator, boron-KNO<sub>3</sub> was ignited in the combustion chamber. The pellet was fired in a test chamber by igniting the conventional ignitor.

Other pellets which have been prepared comprise (1) 60 percent by weight Na N<sub>3</sub>, 15 percent by weight sulfur and 25 percent by weight Na<sub>2</sub> CO<sub>3</sub>; and (2) 61 percent by weight Na N<sub>3</sub>, 15 percent by weight sulfur and 24 percent by weight Ca CO<sub>3</sub>.

Obviously, numerous modifications and variations of the present invention are possible in light of the above techniques. It is therefore to be understood that within the scope of the appended claims the invention may be practiced otherwise than as specifically described herein.

What is claimed as new and desired to be secured by Letters Patent of the United States is:

1. A solid, nitrogen generating composition consisting essentially of (1) an azide selected from the group consisting of sodium azide, lithium azide and mixtures thereof and (2) sulfur.

2. The composition of claim 1 wherein said azide is sodium azide.

3. The composition of claim 1 which additionally contains a substance or mixture of substances which can produce CO<sub>2</sub>.

4. The composition of claim 3 wherein said substance is a carbonate.

5. The composition of claim 1 wherein said azide and said sulfur are present in about stoichiometric quantities.

6. The composition of claim 3 wherein said azide and said sulfur are present in about stoichiometric quantities.

7. The composition of claim 1 wherein the quantity of either said azide or said sulfur is not less than about 20 percent of the stoichiometric quantity.

10 8. The composition of claim 3 wherein the quantity of either said azide or said sulfur is not less than about 20 percent of the stoichiometric quantity.

9. The composition of claim 1 wherein the quantity of said azide or said sulfur is not less than about 75 percent of the stoichiometric quantity.

10 10. The composition of claim 3 wherein the quantity of either side sulfur or said azide is not less than about 75 percent of the stoichiometric quantity.

11. A method of generating hot nitrogen gas comprising igniting the composition of claim 1.

12. A method of generating hot nitrogen and CO<sub>2</sub> comprising igniting the composition of claim 3.

13. A method of generating hot nitrogen which is capable of use in a gas dynamic laser comprising igniting the composition of claim 5.

14. A method of generating hot nitrogen and CO<sub>2</sub> which is capable of use in a gas dynamic laser comprising igniting the composition of claim 6.

\* \* \* \* \*

30

35

40

45

50

55

60

65